

June 21, 1927.

1,632,802

G. A. RICHTER

PROCESS OF AND APPARATUS FOR TREATING FIBER

Filed Aug. 10, 1926



Inventor  
George A. Richter  
by *Right from Linby May*  
*Attys.*

Patented June 21, 1927.

1,632,802

# UNITED STATES PATENT OFFICE.

GEORGE A. RICHTER, OF BERLIN, NEW HAMPSHIRE, ASSIGNOR TO BROWN COMPANY, OF BERLIN, NEW HAMPSHIRE, A CORPORATION OF MAINE.

## PROCESS OF AND APPARATUS FOR TREATING FIBER.

Application filed August 10, 1926. Serial No. 128,398.

This invention relates to a process of treating fiber with a chemical solution, and has for its object to provide a process of treating such fiber in a continuous, efficient 5 and economical manner.

After fiber has been liberated by suitable digestion from wood chips or other cellulose-bearing material, it is frequently desired further to treat such fiber with a chemical solution. For example, it may be desired to treat raw sulphite fiber with a solution 10 of caustic soda to effect a removal of the non-alpha cellulose constituent present therein and thus to produce a fiber containing 15 a high percentage of alpha or resistant cellulose.

If such alkaline treatment is carried out under the proper conditions for the requisite period of time, the resultant fiber will contain upward of 93% alpha cellulose, and is bleachable to a high degree of whiteness with a low strength bleach solution. Such "alpha" or purified cellulose fiber is suitable 20 for use as a new rag or cotton fiber substitute in the manufacture of high grade papers and the preparation of cellulose derivatives. In commercial practice, the chemical present in the spent treating liquor is recovered. In my application for patent, 25 Serial No. 26,361, filed April 28, 1925, I have described a method of economically recovering such chemical. The method therein set forth, however, is dependent upon the use of a raw fiber which has been dried or 30 concentrated to a consistency of, say 50% before alkaline treatment. Consequently a 10% to 12% raw fiber resulting from washing and screening such fiber after its liberation must be concentrated as by passage 35 through a high pressure thickener, press rolls, or the like.

One feature of the process of the present invention is that the chemical present in the spent liquor may be recovered without 40 requiring such high concentration of raw fiber, thus eliminating the necessity of a high pressure thickener or the like. Another feature is that the fiber is washed free from treating chemicals simultaneously with the 45 treatment. Still another feature is that fiber stocks of different water contents may be subjected to treatment. This alkaline or other chemical treatment may be carried out at an elevated temperature, and the heat and

chemical content of the spent liquor conserved.

In accordance with the process of the present invention, the chemical treatment of the fiber takes place while such fiber is being passed through and washed in continuous, 65 counter-current flow. This may be done in apparatus of the general type shown and described in United States Letters Patent No. 1,421,664, issued July 4, 1922, to Brown, Moore, Parker and Martinson. A series of 70 treating baths gradually increasing in concentration of treating chemical from substantially only water at one end of the apparatus to a solution of maximum chemical concentration at an intermediate portion 75 thereof and then gradually decreasing in concentration from the intermediate portion to substantially only water at the other end thereof, is maintained in the apparatus. Water is continuously introduced into one 80 end of the apparatus, and a flow of solution is produced from bath to bath toward the other end of the apparatus, from which water is discharged, and into which fiber to be treated is continuously passed through 85 the apparatus in countercurrent flow to the water. A volume of spent solution containing the chemical being spent is continuously withdrawn from and sufficient fresh chemical solution to make up mechanical losses 90 and to replace chemical in the solution being withdrawn is continuously introduced into the intermediate portion of the apparatus.

For a more complete understanding of this invention, reference may be had to the 95 accompanying drawings, wherein

Figure 1 represents somewhat diagrammatically and conventionally a section through an apparatus for carrying out the process of the present invention.

Figure 2 represents a fragmentary section through an apparatus which is lengthened intermediate its ends.

The apparatus comprises a series of sections, each consisting of a storage tank containing a pool of treating solution, and a treating tank associated therewith and located thereabove. The treating solution in the successive storage tank flows in a direction opposite to the flow of the fiber. These 105 tanks are indicated as 1, 2, 3, 4, 5, 6, 7, 8, 9 and 10, in the direction of solution flow. The solution overflows a series of partitions

11 placed between the tanks and gradually decreasing in height from the tank 1 to the tank 10 so that a substantially continuous flow of solution from the tank 1 to the tank 5 10 results.

The treating tanks are designated as 1<sup>a</sup>, 2<sup>a</sup>, 3<sup>a</sup>, 4<sup>a</sup>, 5<sup>a</sup>, 6<sup>a</sup>, 7<sup>a</sup>, 8<sup>a</sup>, 9<sup>a</sup> and 10<sup>a</sup>, in the direction of the flow of fiber. Each treating tank is divided into two compartments. 10 First, there is a thickening compartment 12, in which rotates a straining cylinder 13, on which the fiber is deposited and through which the treating solution passes and is returned by a pipe 14 to the corresponding 15 storage tank. The fiber deposited on the straining cylinder is squeezed and thickened by a couch roll 15 acting on the cylinder. The fiber is removed from the cylinder and deposited in an agitating compartment 12<sup>a</sup> 20 containing the treating solution, by a scraper 16 acting against the cylinder and stationed on a partition 17 dividing the thickening and agitating compartments. A supply of solution is maintained in each treating tank by 25 withdrawing solution from the corresponding storage tank by a pump 27 and delivering it through a pipe 28 into the agitating compartment. The fiber is agitated in the solution maintained in the treating 30 compartment, by a pair of agitators 18, and flows over a partition 19 into the next adjacent thickening compartment. There is thus a constant circulation of the treating solution from each storage tank, through the 35 agitating compartment of the treating tank, and thence through the straining cylinder back to its storage tank.

The fiber is introduced into the first treating tank 1<sup>a</sup> through a pipe 22, and is withdrawn 40 at the other end of the apparatus from the treating tank 10<sup>a</sup>, through a pipe 23. The treating solution is introduced into the treating tank 5<sup>a</sup> through a pipe 25, and water is introduced into the storage tank 1 45 through a pipe 24 and withdrawn from the storage tank 10 through a pipe 26.

Where a raw fiber, e. g., unbleached sulphite, is to be purified into fiber of high alpha cellulose content, the treating solution 50 may be a solution of caustic soda or equivalent compound. The raw fiber may be delivered into the apparatus, as it comes from the washing and screening operations, as, say, a 10% to 12% aqueous pulp suspension. 55 As it passes through the successive treating tanks toward the center of the apparatus, the water associated therewith is displaced by a caustic soda solution of increasing strength so that it acquires a maximum 60 caustic soda concentration when it reaches the treating tank 5<sup>a</sup> into which the caustic soda solution is introduced. On passing forwardly from the tank 5<sup>a</sup>, the caustic soda solution associated with the fiber is displaced by a solution of progressively de-

creasing strength, so that when the fiber is discharged from the last treating tank 10<sup>a</sup>, the solution is substantially entirely displaced by water.

Operation may be initially commenced by 70 maintaining the volume of caustic soda solution continuously delivered into the treating tank 5<sup>a</sup> and the volume of wash water continuously introduced into the storage tank 1 substantially equal to the volume of water 75 associated with the raw fiber. The apparatus is controlled to discharge a fiber having a water content equal to that of the raw fiber. Substantially only water is discharged through the outlet pipe 26. After the equilibrium concentration of caustic soda has been attained in the tanks, only sufficient caustic soda solution to make up sodium constituent spent and contained in spent solution bled off from the storage tank 5 through 80 a valved pipe 29 and to make up mechanical losses, need be introduced into the treating tank 5<sup>a</sup>. The volume of wash water introduced into the storage tank 1 is then maintained substantially equal to the water content of the raw fiber as it is introduced and the water discharged through the outlet pipe 26 so that the concentration of active or unspent caustic soda in each of the storage 85 and treating tanks remains substantially constant during the continuous operation of the apparatus. The flow bled off through the pipe 29 is regulated to provide for the withdrawal of the solution, the sodium constituent of which has been spent by reaction with the non-alpha cellulose constituent of the fiber so that accumulation of dissolved organic matter in the apparatus is prevented.

Of course, some unspent sodium constituent is necessarily drawn off, also. This bleed 105 solution may be concentrated, incinerated and smelted, as usual, for the recovery of the sodium constituent.

The process may be considered as comprising two steps, during both of which a 110 dissolving and removal of the non-alpha cellulose constituent of the raw fiber by the caustic soda solution is effected. First, the displacement of the water content of the raw fiber by a solution of caustic soda occurs and then the displacement of the solution of caustic soda by water. Consequently, substantially all the treating solution except that drawn off through the pipe 29 is maintained within the apparatus—substantially only water accompanying the purified fiber discharged through the pipe 23 at one end of the apparatus, and substantially only water being discharged through the outlet pipe 26 at the opposite end thereof. If the treatment is carried out at an elevated temperature as by introducing steam into the central pool maintained in the storage tank 6, the heat content (except for that of the bleed solution), in addition to the 120 125 130

chemical content of the solution, is maintained within the apparatus.

When a concentrated solution of caustic soda is employed in treating the fiber, only 5 a relatively short treating period, say, five to ten minutes, at about room temperature, is necessary to produce an alpha fiber having characteristics rendering it especially applicable for viscose preparation.

10 When a relatively dilute solution of caustic soda is employed in treating the fiber, a longer treating period and an elevated temperature are necessary to produce fiber of the desired alpha cellulose content. The 15 time of treatment may be prolonged by operating the apparatus at lower capacity or by constructing one or more of the intermediate storage and corresponding treating tanks of the apparatus longer than the others. Figure 2 shows an apparatus the central section of which is provided with a treating tank, the agitating compartment of which is about four times the length of the other treating compartments and which is 20 shown provided with four pairs of agitators. A longer period of treatment is thus permitted at the section of the apparatus where the solution is strongest and the rate of fiber purification greatest.

25 It is evident that, if desired, a certain amount of bleach liquor or other equivalent oxidizing liquor may be introduced with the caustic soda solution into the tank 5<sup>a</sup> to aid in the purification of the fiber.

30 While the process of the present invention has been described in connection with treatment of raw fiber to purify the same, it is obvious that this is illustrative only, and that the process may be practised to 35 effect a treatment of fiber with other chemical solutions.

What I claim is:

1. A process of treating fiber with a chemical solution and washing the same, which 40 comprises maintaining a series of treating baths, introducing fiber into an end bath and passing said fiber from bath to bath toward the other end bath, introducing water into the other end bath and the chemical solution into an intermediate bath, and 45 producing a flow of water from bath to bath in countercurrent flow to that of the fiber.

2. A process of treating fiber with a chemical solution and washing the same, which 50 comprises maintaining a series of treating baths gradually increasing in concentration of treating chemical from substantially only water at one end of the series and toward an intermediate bath thereof, and then 55 gradually decreasing in concentration from the intermediate bath to substantially only water at the other end thereof, introducing fiber into an end bath and passing said fiber from bath to bath toward the other 60 end bath, introducing water into the other 65

end bath and a chemical solution into the intermediate bath, and producing a flow of water from bath to bath in countercurrent flow to that of the fiber.

3. A continuous process of treating fiber 70 with a chemical solution and washing the same, which comprises continuously feeding the fiber to and agitating it in a series of baths gradually increasing in concentration of treating chemical from substantially only 75 water at one end of the series toward an intermediate bath thereof, and gradually decreasing in concentration from the intermediate bath to substantially only water at the other end thereof, continuously introducing 80 water into the last bath of the series and treating solution into an intermediate bath, and causing the water to flow in opposite direction to that of the fiber through such series of baths. 85

4. A continuous process of removing non-alpha cellulose constituents from an aqueous, raw fiber suspension, which comprises continuously feeding the raw fiber suspension to and agitating it in a series of alkaline 90 baths gradually increasing in concentration of alkali from substantially only water at one end of the series toward an intermediate bath thereof, and gradually decreasing in concentration from the intermediate bath to 95 substantially only water at the other end thereof, continuously introducing water into the last bath of the series and alkaline solution into an intermediate bath, and causing the water to flow in opposite direction to the flow of the fiber through such series of baths. 100

5. A continuous process of removing non-alpha cellulose constituent from an aqueous raw fiber suspension, which comprises continuously feeding the fiber suspension to and agitating it in a series of alkaline baths gradually increasing in concentration of alkali from substantially only water at one end of the series toward an intermediate 105 bath thereof, and gradually decreasing in concentration from the intermediate bath to substantially only water at the other end thereof, continuously introducing water into the last bath of the series in amount equal 110 to the water content of the raw fiber suspension and an alkaline solution into an intermediate bath containing alkali in amount sufficient to make up mechanical losses and alkali being spent by reaction, causing the 115 water to flow in opposite direction to that of the fiber through such series of baths, and regulating the relative flow of the materials to discharge substantially only an aqueous suspension of high alpha cellulose fiber 120 at one end of the series and water at the other end of the series. 125

6. A continuous process of removing non-alpha cellulose constituent from an aqueous raw fiber suspension, which comprises con- 130

- tinuously feeding the fiber suspension to and agitating it in a series of alkaline baths gradually increasing in concentration of alkali from substantially only water at one end of the series toward an intermediate bath thereof, and gradually decreasing in concentration from the intermediate bath to substantially only water at the other end thereof, continuously introducing water into the last bath of the series in amount equal to the water content of the raw fiber suspension being introduced and an alkaline solution into an intermediate bath containing alkali in amount sufficient to make up mechanical losses and alkali being spent by reaction, causing the water to flow in opposite direction to that of the fiber through such series of baths continuously bleeding off spent solution from the intermediate bath, and regulating the relative flows of the materials to discharge substantially only an aqueous suspension of high alpha cellulose fiber at one end of the series and water at the other end of the series.
7. A process of treating a fiber suspension with a chemical solution and washing the same, which comprises maintaining a series of pools of the solution, producing a flow of solution successively from pool to pool, circulating solution from each pool to a treating bath, supplying water to an end pool and chemical solution to an intermediate treating bath, feeding the fiber suspension through the successive baths in a direction opposite to the flow of the water, agitating the fiber in said baths, removing a portion of the solution from said fiber before it is fed from one bath to another, circulating such liquor to the corresponding pool, and regulating the relative flow of the materials to discharge substantially only an aqueous fiber suspension at one end of the series and water at the other end of the series.
8. A process of treating a fiber suspension with a chemical solution and washing the same, which comprises maintaining a series of treating baths, introducing fiber into an end bath and passing said fiber from bath to bath toward the other end bath, agitating the fiber in said baths, thickening said fiber before it is fed from one bath to another, introducing water into the other end bath, introducing treating solution into an intermediate bath, and producing a flow of water from bath to bath in countercurrent flow to that of the fiber.
9. An apparatus for chemically treating and washing fiber, comprising a plurality of sections arranged in series, each section comprising a storage tank containing a pool of treating solution and a treating tank containing a bath of treating solution, means at each section for causing a circulation of solution from the storage tank to the treating tank and thence back to the storage tank, means for passing the fiber into an end treating tank and from one treating tank to the adjacent treating tank, means for introducing water into the storage tank at the opposite end and for causing a flow of water from one storage tank to an adjacent storage tank in opposite direction to the passage of the fiber, and means for introducing treating solution into a treating tank intermediate the ends of said apparatus and for withdrawing solution from a storage tank intermediate the ends of said apparatus.
- In testimony whereof I have affixed my signature.
- GEORGE A. RICHTER.